

# UNITED STATES PATENT OFFICE.

NAPOLEON G. PETINOT, OF NEW YORK, N. Y., ASSIGNOR TO UNITED STATES ALLOYS CORPORATION, OF NEW YORK, N. Y., A CORPORATION OF NEW YORK.

## METHOD OF TREATING IRON OR STEEL.

1,252,023.

Specification of Letters Patent.

Patented Jan. 1, 1918.

No Drawing.

Application filed March 7, 1917. Serial No. 152,980.

To all whom it may concern:

Be it known that I, NAPOLEON G. PETINOT, a citizen of the United States of America, and a resident of the city, county, and State 5 of New York, have invented a new and useful Method of Treating Iron or Steel, of which the following is a full, clear, and exact description.

My invention relates generally to the treatment of iron or steel and more particularly to a treatment in which the slag inclusions in the metal are removed. The general object of my invention is to treat molten iron or steel with an alloy, which will, when oxidizing, form fluid combinations with the slag or oxids of the metal and thus permit their ready escape from the molten mass.

It is well known to those skilled in the art, that the treatment of iron or steel, with ferro-titanium, greatly improves their properties. I have found, however, that in the regular practice of treating iron or steel with ferro-titanium, a certain amount of the titanium combines with oxygen existing in the iron or steel either as free oxygen or combined as oxids, and forms titanium-oxid. This titanium-oxid has a very high melting point and does not become fluid enough to be liberated from the molten mass at the 30 temperature of the molten iron or steel, but only becomes pasty and is, therefore, more or less entrapped in the iron or steel, as such, or is combined with particles of slag in the metal.

I have discovered that by introducing silicon in the alloy in certain definite proportions and then using this alloy for the treatment of iron or steel, results are had which are superior to those heretofore attained.

I am aware that certain patents have been issued on alloys for the treatment of iron or steel where titanium and silicon are used, but in these particular patents it is the desire of the inventor to retain a certain portion of these materials in the finished product. In my process, I use an alloy which has just enough titanium and silicon in it to make the imprisoned slag or oxids fusible, and it is very important that the ratio between the silicon and titanium be exact or they will have a high melting point and the desired results will not be obtained.

I have found that iron or steel, which is treated with ferro-titanium and which 55 contains at least 0.1 per cent. of silicon, results in a much better product than iron or

steel which does not contain the silicon. The silicon in the iron or steel just referred to, is derived from ferro-silicon which, in present practice, is added to the ladle when the steel 60 or iron is tapped from the furnace. Part of the silicon thus added is oxidized to silica, thus forming a slag which is left in the ladle after the steel or iron is poured off.

In the experiments which led to my invention, I took some of this silica of slag, found in the bottom of the ladle, after teeming a basic heat, reduced it to a fine powder and mixed with it to 50 per cent. of pure titanic oxid. The melting point of this mixture, I discovered, was very high. I then made other mixtures of silica or slag and titanic oxid in which the amounts of silica varied from 10 per cent. to 50 per cent, and among these I found one with a low melting 70 point. This latter mixture was one in which the weight of silica was 15 per cent. of the weight of the titanic oxid.

I, therefore, made an alloy of iron, titanium and silicon so proportioned that, 80 when it is used to treat a ferro-metal, the oxids thus formed are in such proportions that their mixture, when combined with any slag in the metal, is far more fusible than the mixtures obtained when the ferro-metal 85 is treated with only ferro-titanium.

It should be observed that my invention does not have for its object to provide an alloy designed to effect the melting point of all of the slag of any mass of molten 90 metal taken from the furnace, but merely that portion of the slag or oxids which are scattered throughout and imprisoned within the mass.

In carrying out my invention, if the alloy 95 is used to treat steel, which contains iron oxid, the following reactions will take place, simultaneously:



If the titanium and silicon are in proper proportions, the titanic oxid and silica formed will combine with the slag or oxids which are imprisoned in the mass of molten 105 steel, thus forming silico-titanates, which have low melting points. These silico-titanates, on account of their low melting points form relatively mobile liquids which readily escape from the molten steel, thus producing 110 a superior steel. The treatment of steel with my alloy is far superior to the treat-

ment of steel with ferro-titanium or ferro-silicon separately, because, with my alloy, the titanic oxide and silica are formed simultaneously, and in immediate proximity to 5 one another and the slag or oxide, which it is desired to remove from the molten metal.

As hereinbefore stated, it is essential that the proportions between the silicon and titanium be exact, for if the percentage of titanium is greater than a certain definite amount, the combination will have a high melting point. I have found that in order to successfully carry out my process, I must have an alloy which contains from 15 per 15 cent. to 25 per cent. titanium, 3 per cent. to 5 per cent. silicon, and carbon in various amounts. In this alloy, the silicon exists as iron silicid and the carbon partly combined as a double carbid of iron and titanium and 20 partly in the graphitic state. The graphitic carbon contained in the alloy is doubtless produced by the presence of the silicon, which, as is well known to metallurgists, tends to throw carbon out of the combination 25 and into the graphitic state.

In carrying out my process, I add the alloy specified above to the molten iron or steel in such proportions that the oxygen contained in the metal oxidizes the titanium 30 and silicon in the alloy and forms titanic oxide and silica, which might combine with

the imprisoned slag or oxids of the molten mass, thus forming very fusible silico-titanates. These titanates, on account of their great fluidity, rapidly escape to the surface 35 of the metal, thus relieving the molten mass of the slag and oxids and forming a greatly improved product. As hereinbefore stated, the proportion of the alloy to the molten mass is such that none of the titanium or 40 silicon or their oxids are left in the steel or iron.

Having thus described my invention what I claim is:

1. A method of treating iron or steel comprising the addition thereto, while molten, of an alloy of iron, titanium and silicon, in which iron is in the largest proportion and silicon is in such less proportion to the titanium that on oxidation, a low fusing silico-titanate is formed. 45

2. A method of treating iron or steel comprising the addition thereto, while molten, of an alloy of iron, titanium and silicon, in which the iron amounts to from 69% to 80% 50 of the total weight of the alloy, and in which the silicon is about one-quarter of the weight of the titanium in the alloy. 55

In testimony whereof, I have hereunto signed my name.

NAPOLEON G. PETINOT.